

1

3,642,972

## PROCESS OF PRODUCING NONWOVEN FABRICS USING AZIRIDINE-MODIFIED POLYURETHANE BONDING AGENT

Howard L. Needles, Davis, and William L. Wasley, Berkeley, Calif., assignors to the United States of America as represented by the Secretary of Agriculture

No Drawing. Filed Nov. 19, 1969, Ser. No. 882,407

Int. Cl. D04h 1/00

U.S. Cl. 264—123

5 Claims

### ABSTRACT OF THE DISCLOSURE

Non-woven fabrics which combine good tensile strength with porosity, air-permeability, flexibility, softness, and the appearance and handle of a woven fabric. Products of the invention, although made from wool, do not shrink when washed in aqueous soap or detergent formulations. Example: An aziridine-modified polyurethane is deposited on wool fibers which are then arranged in the form of a thin web and cured at a temperature of about 100–170° C. under a pressure of about 1000–5000 p.s.i.

A non-exclusive, irrevocable, royalty-free license in the invention herein described, throughout the world for all purposes of the United States Government, with the power to grant sublicenses for such purposes, is hereby granted to the Government of the United States of America.

This invention concerns the production of fabrics of the non-woven category, that is, fabrics wherein the fibrous elements which comprise the structure are joined by bonding with an adhesive composition rather than by weaving or knitting. More particularly, the invention concerns the provision of non-woven fabrics which exhibit many of the characteristics of typical woven fabrics. Thus, the products of the invention combine good tensile strength with porosity, air-permeability, flexibility, softness, and the appearance and handle of a woven fabric. Moreover, although the products of the invention are made from wool, they do not shrink when washed in aqueous soap or detergent formulations. Further objects and advantages of the invention will be evident from the following description wherein parts and percentages are by weight unless otherwise specified.

Certain non-woven fabrics are now available in commerce. These products consist of a skeleton of textile fibers bonded together by such resinous materials as polyvinyl esters, polyacrylates, polystyrene, polyvinylidene, and copolymers of these substances and the like. A common property of these known products is that they are stiff. Indeed, they are used as stiffening materials for lapels, collars, and similar garment parts. Another disadvantage of the known non-woven fabrics is that they cannot withstand the stresses encountered in laundering. When subjected to the usual agitation in soap (or detergent) and hot water formulations they are ruptured or even disintegrated. For example, Nottebohm (U.S. Pat. 2,719,803) explains that non-woven fabrics cannot be washed without damage, and to remedy this problem he finds it necessary to protect an inner layer of non-woven fabric by laminating it with outer layers of conventional woven fabrics.

A primary object of the invention is the provision of novel products which avoid the problems outlined above, that is, the provision of products which, among other advantages, are free from stiffness and which are stable to washing in aqueous media.

In accordance with the invention, wool fibers are first

2

coated with an aziridine bonding agent (as herein-after described). A preferred technique involves dissolving the aziridine in an inert, volatile solvent and applying the resulting solution to the wool fibers. Typical of the solvents which may be used are benzene, toluene, xylene, dioxane, diisopropyl ether, dibutyl ether, butyl acetate, chlorinated hydrocarbons such as chloroform, carbon tetrachloride, ethylene dichloride, trichloroethylene, 1,3-dichlorobenzene, fluorohydrocarbons such as benzotrifluoride, 1,3-bis(trifluoromethyl) benzene, etc., petroleum distillates such as petroleum naphthas, etc. Usually it is preferred to use the aziridines in the form of aqueous emulsions. These can be prepared by customary techniques—agitation of the aziridine with water and a conventional emulsifying agent such as an alkylphenoxy-poly(ethyleneoxy) ethanol, polyoxyethylene sorbitan monopalmitate, polyoxyethylene lauryl ether, polyoxyethylene lauryl ether, polyoxyethylene-polyoxypropylene stearate, sorbitan monopalmitate, sorbitan monolaurate, and the like. The concentration of the aziridine in the dispersion—this last term being herein employed in a generic sense to include solutions and emulsions—is not critical and may be varied depending on such circumstances as the solubility characteristics of aziridine, the amount of aziridine to be deposited on the fibers, the viscosity of the dispersion, etc. In general, a practical range of concentration would be from about 1% to about 25%. The dispersion may be distributed on the textile material by any of the usual methods, for example, by spraying, brushing, padding, dipping, etc. A preferred technique involves immersing the fibers in the dispersion and then passing them through squeeze rolls to remove the excess of liquid. Such techniques as blowing air through the treated textile may be employed to reduce the amount of liquid which exists in interstices between fibrous elements. In any case, the conditions of application are so adjusted that the textile material contains the proportion of aziridine desired. Generally, the amount of aziridine is about from 5 to 25%, based on the weight of the wool fibers but it is obvious that higher proportions may be used for special purposes.

After application of the aziridine, the treated fibers are dried to remove the solvent or dispersing vehicle. The drying may be at room temperature, or somewhat elevated temperatures, for example, up to about 60° C. The fibers are then arranged to form a thin sheet or web. The fibers may be arranged parallel, in a criss-cross pattern, or randomly. For best results the fibers are arranged in superposed layers with the fibers of each layer at an angle to the fibers of adjacent layers, thus to provide a multiplicity of points of contact between individual fibers.

The web or sheet of aziridine-treated fibers is then subjected to a temperature of about 100–170° C. while under a pressure of about 1000–5000 p.s.i. applied, for example, by heated platens or the like. By this heating and pressurizing step the aziridine is cured so that the fibers are permanently bonded into a unitary structure. Also, at the initiation of the curing step, the aziridine which has been applied to the fibers is fused and migrates to points where individual fibers intersect. This means that after the aziridine has been insolubilized (cured) the fibers are adhered mainly at crossing points rather than being continuously adhered all along their lengths. Such a result is, of course, advantageous as it yields a product which is like a fabric (i.e., porous, resilient, etc.) and not impermeable and limp like a plastic foil or sheet. Another important result of the curing step is that the aziridine is chemically bonded to the wool fibers. Although the mechanism of this bonding has not been identified, it is believed to involve chemical combination of the

aziridine with active radicals in the wool molecules, these active radicals including carboxyl, hydroxyl, amino, and thiol groups. This chemical combination of the aziridine with the wool fibers is of advantage as it adds to the durability of the products, particularly their ability to be washed without shrinking or other damage.

The non-woven fabrics prepared by the technique described above have many advantages properties. They are porous, air-permeable, soft, flexible, and resilient. Thus, unlike prior art products they exhibit most of the properties of the wool fibers themselves so that they are eminently suitable for preparing all kinds of garments. A particularly important advantage of our products is that they can be washed with the usual soap (or detergent) and hot water formulations without rupture, indeed without even shrinking. Moreover, the products display an excellent resistance to wrinkling and creasing.

The aziridines used in accordance with the invention are those described and claimed in the co-pending application of Allen G. Pittman and William L. Wasley, Ser. No. 675,038, filed Oct. 13, 1967, now Pat. 3,542,505. They may be aptly described as aziridine-modified polyurethanes, and have the structure



wherein:

A is the residue of a polyether polyol or polyester polyol having a valence of  $n$ ,

R is a hydrocarbon radical containing at least two carbon atoms,

R' is hydrogen, halogen, lower alkoxy, or a radical of the structure



R'' is hydrogen or a lower alkyl radical,

n is an integer from 2 to 10, and

x is an integer from 1 to 2.

The aziridine derivatives of the invention are prepared by reacting an alkylene imine, such as ethylene, propylene, or butylene imine, with a polyether (or polyester) polyurethane containing free isocyanate groups. This simple reaction establishes the desired aziridine-modification of the starting polymer. A typical, but by no means limiting, example of the synthesis is illustrated below:

(In the formulas,  $m$  represents the number of tetramethylene repeating units. This may range, for example, about from 5 to 50.)

The reaction is carried out at about 10 to 40° C., and under essentially anhydrous conditions to avoid hydrolysis of the isocyanate groups. The alkylene imine is supplied in excess to ensure conversion of all isocyanate groups to aziridine groups. It is evident from the formulas above that modification in the aziridine rings can be effected by selection of the alkylene imine reactant. For example, if propylene imine is used instead of ethylene imine, the aziridine rings will be of the structure



In other words, in this case R'' (in Formula I) is methyl.

Referring to Formula I, above, it is evident that selection of the polymer intermediate—the polyether or polyester polyurethane containing free isocyanate groups—will determine the values of A, R, R', n, and x. The preparation of these intermediates is well known in the art; they are widely used in the production of urethane foams for padding and insulation applications, and in the production of elastomers. Although the preparation of these intermediates forms no part of the present invention, this subject will be explained below to illustrate the wide range of intermediates which may be employed in producing the aziridine derivatives of the invention. Thus, for the purposes of the invention, the intermediate may be any polyether or polyester polyurethane which contains at least two free NCO groups per polymer molecule. Preferred are the polymer intermediates having a molecular weight of at least 500, more preferably those having a molecular weight of at least 1000. Also, it is generally preferred to use the polyether-based polymers, for example, the NCO-containing polyurethanes derived from polyalkylene ether glycols such as polyethylene ether glycols, polytrimethylene ether glycols, polytetramethylene ether glycols, polypropyleneether glycols, and the like.

#### THE POLYMER INTERMEDIATES

Polyether (or polyester) polyurethanes containing free isocyanate groups useful as intermediates for the present invention may be prepared, as well known in the art, by reacting a polyether (or polyester) polyol with a polyisocyanate, using an excess of the latter to ensure provision of free isocyanate groups in the product. A typical, but by no means limiting, example is illustrated:





Isocyanate-terminated polyether polyurethane

(In the above formulas,  $m$  represents the number of tetramethyleneether repeating units. This may range, for example, about from 5 to 50.)

Representative examples of polyisocyanates which may be employed for reaction with the polyether (or polyester) polyol include:

toluene-2,4-diisocyanate  
 toluene-2,6-diisocyanate  
 commercial mixtures of toluene-2,4 and 2,6-diisocyanates  
 ethylene diisocyanate  
 ethylidene diisocyanate  
 propylene-1,2-diisocyanate  
 cyclohexylene-1,2-diisocyanate  
 cyclohexylene-1,4-diisocyanate  
 m-phenylene diisocyanate  
 3,3'-diphenyl-4,4'-biphenylene diisocyanate  
 4,4'-biphenylene diisocyanate  
 3,3'-dichloro-4,4'-biphenylene diisocyanate  
 1,6-hexamethylene diisocyanate  
 1,4-tetramethylene diisocyanate  
 1,10-decamethylene diisocyanate  
 1,5-naphthalene diisocyanate  
 cumene-2,4-diisocyanate  
 4-methoxy-1,3-phenylene diisocyanate  
 4-chloro-1,3-phenylene diisocyanate  
 4-bromo-1,3-phenylene diisocyanate  
 4-ethoxy-1,3-phenylene diisocyanate  
 2,4'-diisocyanato diphenylether  
 5,6-dimethyl-1,3-phenylene diisocyanate  
 2,4-dimethyl-1,3-phenylene diisocyanate  
 4,4'-diisocyanato diphenylether  
 benzidine diisocyanate  
 4,6-dimethyl-1,3-phenylene diisocyanate  
 9,10-anthracene diisocyanate  
 4,4'-diisocyanato dibenzyl  
 3,3-dimethyl-4,4'-diisocyanato diphenylmethane  
 2,6-dimethyl-4,4'-diisocyanato diphenyl  
 2,4-diisocyanato stilbene  
 3,3'-dimethyl-4,4'-diisocyanato diphenyl  
 3,3'-dimethoxy-4,4'-diisocyanato diphenyl  
 1,4-anthracene diisocyanate  
 2,5-fluorene diisocyanate  
 1,8-naphthalene diisocyanate  
 2,6-diisocyanato benzofuran  
 2,4,6-toluene triisocyanate, and  
 p,p',p''-triphenylmethane triisocyanate.

It is evident that the selection of the polyisocyanate reactant will determine the values of  $R$  and  $R'$  in Formula I. For example, where the reactant is a hydrocarbon diisocyanate,  $R$  will be a hydrocarbon radical and  $R'$  will represent a hydrogen atom forming part of said hydrocarbon radical. Where the reactant contains a substituent such as chlorine or methoxy—as would be the case with, for example, 4-chloro-1,3-phenylene diisocyanate or 4-methoxy-1,3-phenylene diisocyanate— $R$  will be the hydrocarbon residue of the reactant and  $R'$  will be the substituent—chlorine or methoxy in the given examples.

Polyether polyol. The polyether polyol useful for the purposes of the invention may be derived from any of a wide variety of polyether polyols, and representative examples of these polyols are described below:

## Polyisocyanate



drocarbon residue of the reactant and  $R'$  will be the substituent—chlorine or methoxy in the given examples.

The polymer intermediates useful for the purposes of the invention may, in turn, be derived from any of a wide variety of polyether polyols and polyester polyols, and representative examples of these polyols are described below:

Among the polyether polyols which may be so used are those prepared by reaction of an alkylene oxide with an initiator containing active hydrogen groups, a typical example of the initiator being a polyhydric alcohol such as ethylene glycol. The reaction is usually carried out in the presence of either an acidic or basic catalyst. Examples of alkylene oxides which may be employed in the synthesis include ethylene oxide, propylene oxide, any of the isomeric butylene oxides, and mixtures of two or more different alkylene oxides such as mixtures of ethylene and propylene oxides. The resulting polymers contain a polyether backbone and are terminated by hydroxyl groups. The number of hydroxyl groups per polymer molecule is determined by the functionality of the active hydrogen initiator. For example, a difunctional alcohol such as ethylene glycol (as the active hydrogen initiator) leads to polyether chains in which there are two hydroxyl groups per polymer molecule. When polymerization of the oxide is carried out in the presence of glycerol, a trifunctional alcohol, the resulting polyether molecules contain an average of three hydroxyl groups per molecule. Even higher functionality—more hydroxyl groups—is obtained when the oxide is polymerized in the presence of such polyols as pentaerythritol, sorbitol, dipentaerythritol, and the like. In addition to those listed above, other examples of polyhydric alcohols which may be reacted with alkylene oxides to produce useful polyether polyols include:

55 propylene glycol  
 trimethylene glycol  
 1,2-butylene glycol  
 1,3-butanediol  
 60 1,4-butanediol  
 1,5-pantanediol  
 1,2-hexylene glycol  
 1,10-decanediol  
 1,2-cyclohexanediol  
 65 2-butene-1,4-diol  
 3-cyclohexene-1,2-dimethanol  
 4-methyl-3-cyclohexene-1,1-dimethanol  
 3-methylene-1,5-pantanediol  
 diethylene glycol  
 70 (2-hydroxyethoxy)-1-propanol  
 4-(2-hydroxyethoxy)-1-butanol  
 5-(2-hydroxypropoxy)-1-pentanol  
 1-(2-hydroxymethoxy)-2-hexanol  
 1-(2-hydroxypropoxy)-2-octanol  
 75 3-allyloxy-1,5-pantanediol

2-allyloxymethyl-2-methyl-1,3-propanediol  
 [(4-pentyloxy)methyl]-1,3-propanediol  
 3-(o-propenylphenoxy)-1,2-propanediol  
 thiodiglycol  
 2,2'-[thiobis(ethyleneoxy)]diethanol  
 polyethyleneether glycol (molecular weight about 200)  
 2,2'-isopropylidenebis(p-phenyleneoxy)diethanol  
 1,2,6-hexanetriol  
 1,1,1-trimethylolpropane  
 3-(2-hydroxyethoxy)-1,2-propanediol  
 3-(2-hydroxypropoxy)-1,2-propanediol  
 2,4-dimethyl-2-(2-hydroxyethoxy)methylpentanediol-1,5  
 1,1,1-tris[(2-hydroxyethoxy)methyl]ethane  
 1,1,1-tris[(2-hydroxypropoxy)methyl]propane  
 triethanolamine  
 triisopropanolamine  
 resorcinol  
 pyrogalol  
 phloroglucinol  
 hydroquinone  
 4,6-di-tertiarybutyl catechol  
 catechol  
 orcinol  
 methylphloroglucinol  
 hexylresorcinol  
 3-hydroxy-2-naphthol  
 2-hydroxy-1-naphthol  
 2,5-dihydroxy-1-naphthol  
 bis-phenols such as 2,2-bis-(p-hydroxyphenyl)propane and



bis-(p-hydroxyphenyl)methane  
 1,1,2-tris-(hydroxyphenyl)ethane  
 1,1,3-tris-(hydroxyphenyl)propane.

An especially useful category of polyether polyols are the polytetramethylene glycols. They are prepared by the ring-opening polymerization of tetrahydrofuran, and contain the repeating unit



in the polymer backbone. Termination of the polymer chains is by hydroxyl groups.

The polyester polyols which may be employed as precursors for the aziridines of the invention, are most readily prepared by condensation polymerization of a polyol with a polybasic acid. The polyol and acid reactants are used in such proportion that essentially all of the acid groups are esterified and the resulting chain of ester units is terminated by hydroxyl groups. Representative examples of polybasic acids for producing these polymers are oxalic acid, malonic acid, succinic acid, glutaric acid, adipic acid, pimelic acid, suberic acid, azelaic acid, sebacic acid, brassylic acid, thapsic acid, maleic acid, fumaric acid, glutaconic acid,  $\alpha$ -hydromuconic acid,  $\beta$ -hydromuconic acid,  $\alpha$ -butyl- $\alpha$ -ethylglutaric acid,  $\alpha$ , $\beta$ -diethylsuccinic acid, o-phthalic acid, isophthalic acid, terephthalic acid, hemimellitic acid, trimellitic acid, trimesic acid, mellophanic acid, prehnitic acid, pyromellitic acid, citric acid, benzenepentacarboxylic acid, 1,4-cyclohexanedicarboxylic acid, diglycolic acid, thiodiglycolic acid, dimerized oleic acid, dimerized linoleic acid, and the like. Representative examples of polyols for forming these polymers includes ethylene glycol, 1,3-propylene glycol, 1,2-propylene glycol, 1,4-butylene glycol, 1,3-butylene glycol, 1,2-butylene glycol, butene-1,4-diol, 1,5-pentane diol, 1,4-pentane diol, 1,3-pentane diol, 1,6-hexane diol, hexene-1,6-diol, 1,7-

heptane diol, diethylene glycol, glycerine, trimethylol propane, 1,3,6-hexanetriol, triethanolamine, pentaerythritol, sorbitol, and any of the other polyols listed hereinabove in connection with the preparation of polyether polyols.

- 5 An interesting class of polyester polyols are those which include polyether units so that they may be considered as polyester polyols or as polyether polyols, depending on whether the ester or the ether groups are in majority. The compounds may be produced by the condensation polymerization of any of the above-mentioned polybasic carboxylic acids with a polyalkyleneether glycol—typically, a polyethyleneether glycol having a molecular weight of about 200 to 2000—using the glycol in the required proportion to assure termination by hydroxyl.
- 10 Esters of the hydroxyl-containing acid, ricinoleic acid, form another category of useful polyester polyols. Typically, one can use esters of ricinoleic acid with ethylene glycol, propylene glycol, glycerol, pentaerythritol, diglycerol, dipentaerythritol, polyalkyleneether glycols, and the like. Representative of this category of polyester polyols is castor oil which is composed mainly of the tri-glyceride of ricinoleic acid.
- 15 The invention is further demonstrated by the following illustrative examples.

#### EXAMPLE 1

The aziridine-modified polyurethane used in this instance was prepared as described in Ex. 4 below. It has the structure

A 10% solution of the aziridine-modified polyurethane in toluene was prepared and used to treat wool sliver (a loose assembly of wool fibers). The wool sliver was passed through the solution and then excess liquid removed, using 45 pad rolls to attain an 80–100% wet pick-up of solution. The treated sliver was dried at room temperature. The uptake of aziridine was 8%.

- The dried sliver was cut into 15 cm. long segments (3 grams each) which were spread into 15 x 15 cm., single-ply or 2-ply (crossed), webs between sheets of aluminum foil. The web in each foil was pressed at 2000 p.s.i. and 150° C. for 5 minutes in a hydraulic press. After removal from the press, the foil was removed to yield non-woven fabric samples which weighed approximately 13 mg./cm.<sup>2</sup>.  
 55 The products were very resilient and could be laundered. Various tests were conducted on the samples, the results being tabulated below:

| 60 | Test                              | Direction  | Product |       |
|----|-----------------------------------|------------|---------|-------|
|    |                                   |            | 1-ply   | 2-ply |
|    | Break strength,* dry, lbs.        | {Warp..... | 9.5     | 8.1   |
|    |                                   | {Fill..... | 3.9     | ..... |
|    | Break strength,* wet, lbs.        | {Warp..... | 4.4     | 4.3   |
|    |                                   | {Fill..... | 2.7     | ..... |
|    | Monsanto wrinkle recovery, degree | {Warp..... | 148     | 150   |
|    |                                   | {Fill..... | 149     | 145   |
| 65 | Flexural rigidity, mg.-cm.        | {Warp..... | 984     | 1,090 |
|    |                                   | {Fill..... | 891     | ..... |

\*ASTM test method D-39-49, 1-inch wide strip.

#### EXAMPLE 2

- 70 The procedure described in Example 1 was repeated with the exception that the concentration of the aziridine solutions was increased to give uptakes of the aziridine polymer of 14.4% and 28%. Tests were conducted on the resulting products, these including a shrinkproofing test as follows:

## Accelerotor shrinkage test

This test for shrinkage was conducted in the following way: The samples were milled at 1700 r.p.m. for 2 minutes at 40-42° C. in an accelerotor with 0.5% sodium oleate solution, using a liquor-to-wool ratio of 50 to 1. After this washing operation the samples were measured to determine their area and the shrinkage was calculated from the original area. The accelerotor is described in the American Dyestuff Reporter, vol. 45, p. 685, Sept. 10, 1956. The two-minute wash in this device is equal to about 15 home launderings. Conventional woven wool fabrics when treated in this manner exhibit an area shrinkage of 45 to 50%. The results obtained are tabulated below:

| Test                                                       | Direction | Products        |       |               |       |
|------------------------------------------------------------|-----------|-----------------|-------|---------------|-------|
|                                                            |           | 14.4% aziridine |       | 28% aziridine |       |
|                                                            |           | 1-ply           | 2-ply | 1-ply         | 2-ply |
| Break strength,* dry, lbs. (Warp)                          |           | 22.3            | 11.1  | 21.3          | 17.4  |
|                                                            | (Fill)    | 1.4             | 9.9   | 3.6           | ----- |
| Break strength,* wet, lbs. (Warp)                          |           | 12.7            | 6.6   | 15.1          | 10.2  |
|                                                            | (Fill)    | 1.8             | 6.2   | 2.6           | ----- |
| Air permeability, ft. <sup>3</sup> /ft. <sup>2</sup> /min. |           | 101             | 138   | 189           | 108   |
| Area shrinkage, percent                                    |           | 0               | 1     | 0             | 0     |

\*ASTM test method D-39-49, 1-inch wide strip.

## EXAMPLE 3

The procedure described in Example 1 was repeated with these exceptions: The aziridine was that described in Example 6 below. It has the structure



The curing step was at 150° C., 2000 p.s.i. for 10 minutes. The products had an 11% uptake of the aziridine polymer. Tests on the products are tabulated below:

| Test                                                       | Direction | Product |       |
|------------------------------------------------------------|-----------|---------|-------|
|                                                            |           | 1-ply   | 2-ply |
| Break strength,* dry, lbs. (Warp)                          |           | 7.6     | 4.4   |
|                                                            | (Fill)    | 1.4     | 3.5   |
| Break strength,* wet, lbs. (Warp)                          |           | 4.2     | 3.5   |
|                                                            | (Fill)    | 2.4     | ----- |
| Monsanto wrinkle recovery, degree (Warp)                   |           | 148     | 140   |
|                                                            | (Fill)    | 151     | ----- |
| Air permeability, ft. <sup>3</sup> /ft. <sup>2</sup> /min. |           | 167     | 147   |
| Area shrinkage, percent                                    |           | 0       | 1     |

\*ASTM test method D-39-49, 1-inch wide strip.



The following examples illustrate syntheses of the aziridines useful for the purposes of this invention.

## EXAMPLE 4

## Preparation of aziridine-modified polytetramethyleneether polyurethane

The starting material for this synthesis was a commercial liquid polyurethane having a molecular weight of about 2000 and an isocyanate (—NCO) content of 4.1%. It is believed to have the structure



wherein A' represents the residue of a polytetramethyleneether glycol containing about twenty-five



- 5 Two hundred grams (0.1 mole) of the polyurethane were dissolved in 300 grams of toluene. While stirring the solution, 8 grams (0.2 mole) of ethylene imine were added dropwise. During the addition, the temperature of the solution was not allowed to exceed approximately 40° C. At the end of the addition, an infrared spectrum of the solution revealed no residual NCO groups. This indicated preparation of the desired aziridine derivative.

## EXAMPLE 5

15 The starting material for this synthesis was a commercial liquid polyether polyurethane having a molecular weight of about 850 and an isocyanate (—NCO) content of about 9.5%. It is believed to have the structure.



25 wherein A' represents the residue of a polytetramethyleneether glycol containing about seven



units.



One hundred grams (0.12 mole) of the liquid polyurethane was dissolved in 300 ml. of dry benzene. While stirring, 13 ml. (0.26 mole) of ethylene imine was added at a rate slow enough that the reaction temperature did not rise above 40° C.

## EXAMPLE 6

40 The starting material for the synthesis was a commercial liquid polyether polyurethane having a molecular weight of about 1300 and an isocyanate (—NCO) content of 6.5%. It is believed to have the structure

45



60

One hundred grams (0.077 mole) of the liquid polyurethane was dissolved in 200 grams of dry benzene. To this solution was added 7 grams (0.16 mole) of ethylene imine at a rate slow enough so that the temperature of the reaction mixture did not rise above 35° C. Five minutes after the last of the ethylene imine had been added, the IR spectrum of the reaction mixture showed that no free NCO was present.

## EXAMPLE 7

70 A polypropyleneether glycol of molecular weight about 6000 was reacted with toluene diisocyanate in conventional manner to form an isocyanate-terminated polyurethane. This, in turn, was reacted with propylene imine

## 11

to form an aziridine-modified polyurethane with terminal groups of the structure



Fifty grams of the aziridine-modified polymer—having a molecular weight of 6300–6800 and containing 0.36 to 0.38 milli-equivalents of imine per gram of polymer—was dissolved in 50 grams of benzene and 2 grams of a commercial emulsifier, a polyoxyethylene-polyoxypropylene monostearate, was added. While stirring the solution in a blender, water was gradually added to make 1000 grams of an emulsion.



Having thus described the invention, what is claimed is:

1. A process for preparing a non-woven fabric which comprises



(a) depositing on wool fibers an aziridine-modified polyurethane of the structure



wherein:

A is the residue of a polyether polyol or polyester polyol having a valence of  $n$ ,

R is a hydrocarbon radical containing at least two carbon atoms,

R' is hydrogen, halogen, lower alkoxy, or a radical of the structure



## 12

R'' is hydrogen or a lower alkyl radical,

$n$  is an integer from 2 to 10, and

$x$  is an integer from 1 to 2,

(b) arranging the treated wool fibers into the form of a thin web, and

(c) while constraining the fibers in the form of a thin web, curing the web at a temperature of about 100–170° C. and a pressure of about 1000–5000 p.s.i.

2. The process of claim 1 wherein A is the residue of a polyalkyleneether glycol and  $n$  is 2.

3. The process of claim 1 wherein



15 is the tolylene radical.

4. The process of claim 1 wherein the aziridine-modified polyurethane has the structure



5. The process of claim 1 wherein the aziridine-modified polyurethane has the structure



## References Cited

## UNITED STATES PATENTS

3,542,505 11/1970 Pittman et al. ----- 8—127.6

40 ROBERT F. BURNETT, Primary Examiner  
R. O. LINKER, JR, Assistant Examiner

U.S. Cl. X.R.

45 156—296, 331; 161—157, 170